

## UNITED STATES PATENT OFFICE

WILLIAM ALEXANDER DICKIE AND WILLIAM IVAN TAYLOR, OF SPONDON, NEAR DERBY, ENGLAND, ASSIGNORS TO CELANESE CORPORATION OF AMERICA, A CORPORATION OF DELAWARE

## TEXTILE FABRIC

No Drawing. Application filed August 2, 1929, Serial No. 383,153, and in Great Britain September 28, 1928.

This invention relates to textile fabrics and articles, and comprises fabrics and articles which have a novel appearance by reason of the employment therein of yarns or threads having themselves peculiar and novel characteristics.

Textile fabrics and articles according to the invention are characterized by the employment in the fabric or other textile structure of yarns or threads comprising a number of artificial filaments merged or coalesced to form by their physical union a single unitary filament of larger denier. All the filaments of the yarn or thread may be physically united, so that the yarn or thread is in effect one large unitary filament. Alternatively, the individual filaments of the yarn or thread may be associated into groups, one or more or all of which may be united into unitary filaments. Thus, the filaments may be divided into groups comprising equal or unequal numbers of filaments, and all the groups may be merged or coalesced to form a yarn or thread consisting of unitary filaments of larger denier corresponding to the groups chosen. Or again, one or more equal or unequal groups may be selected from the filaments comprising the yarn or thread and united to produce a yarn or thread consisting of unitary filaments corresponding to the groups selected, and one or more individual filaments. Such yarns or threads consisting entirely of a number of unitary filaments or of one or more unitary filaments and one or more individual filaments may be employed with the unitary filaments, or the unitary and individual filaments, in untwisted form, or they may have imparted to them any desired degree of twist. The yarns or threads may also contain other yarns or threads, or even metallic wires or fine tapes, and such other materials may be secured in the structure of the unitary filaments. Thus, for example, unitary filaments composed of cellulose acetate or other organic derivatives of cellulose may be doubled with or have incorporated in their structure yarns or threads of viscose, nitrocellulose, or cuprammonium artificial silk, or of natural fibres such as silk, cotton, or wool.

The yarns or threads consisting wholly or partly of unitary filaments may be arranged to form figures, patterns or other effects, and they may be employed in the production of fabrics and articles by weaving, knitting, 55 netting, lace-making, or other fabric-forming operations, or in braiding, cording, or other textile operations, and they may be employed alone or in conjunction with yarns or threads consisting of the same artificial filaments or 60 of other natural or artificial filaments or fibres, or with mixed yarns or threads. The unitary filament yarns may, moreover, be doubled or twisted with other yarns.

In fabric-forming operations, the yarns or threads comprising or containing unitary filaments may be arranged to form, for example, bands, stripes, figures, or other designs, or they may be formed, for example into ribbons or bands, being used, say, as weft, on a 70 warp of other yarns or threads of the same or other artificial filaments or of other filaments or fibres.

Unique and pleasing effects are obtained by reason of the different lustre exhibited by 75 the unitary filaments when associated in fabrics or articles with individual filaments, either contained in the same yarns or threads or in other yarns or threads. This effect, may, moreover, be enhanced by dyeing or otherwise colouring the yarns or threads, or the fabrics or articles produced therefrom, the unitary filaments presenting a different appearance from the individual filaments. Cross-dyed effects may be produced in fabrics containing both the unitary filament yarns and yarns of other artificial filaments or of other fibres having a different affinity 80 for the dye-stuff employed, as well as by using unitary filament yarns containing two or more kinds of filaments or fibres having different affinities for the dyestuff. Further, the texture and feel of the fabrics or articles may be modified by the employment of the unitary filaments. 85

As above stated, in yarns or threads containing a number of unitary filaments, or one or more unitary filaments in association with one or more individual or primary filaments, the unitary filaments may vary in denier in 100

accordance with the number of primary filaments united therein. Similarly, when yarns or threads are employed consisting of single unitary filaments, i. e., filaments in which all 5 the filaments have been united to form one larger filament, the effects produced by the introduction or employment of the unitary filaments may be augmented by using unitary filaments of different denier, for example, 10 filaments produced by merging or coalescing either a different number of primary filaments or a similar number of primary filaments themselves of different denier.

The invention is particularly applicable to 15 the use of yarns or threads consisting of or containing unitary filaments composed of cellulose acetate, and also to the use of such filaments in association with yarns or threads of filaments of cellulose acetate as normally used 20 in textile fabric-forming operations, or in association with yarns or threads of other natural or artificial filaments or fibres. The invention may also be applied to the employment in textile fabrics and articles of yarns 25 or threads consisting of or containing unitary filaments composed of other organic derivatives of cellulose, such as cellulose formate, propionate, or butyrate, thiocarbamic or alkoxyl-alkacetyl esters of cellulose, methyl, ethyl, 30 or benzyl cellulose, or the condensation products of cellulose and glycols or other polyhydric alcohols, and also those composed of viscose, nitrocellulose, or cuprammonium artificial silk.

35 Use may be made of the property which nitric acid has for shrinking yarns of cellulose acetate or other organic derivatives of cellulose, by submitting fabrics containing yarns comprising one or more unitary filaments of cellulose acetate or other organic derivative of cellulose to a shrinking treatment with nitric acid, or by employing in the fabrics such yarns which have previously been shrunk by that method.

40 45 What we claim and desire to secure by Letters Patent is:—

1. Textile fabrics comprising in their structure yarns containing at least one unitary filament consisting of a plurality of filaments 50 of cellulose acetate and yarns of fibres different from cellulose acetate coalesced into physical union.

55 2. Textile fabrics comprising in their structure yarns containing at least one unitary filament consisting of a plurality of filaments of cellulose acetate and metallic wires secured in their structure by the coalescing of the cellulose acetate filaments.

60 In testimony whereof we have hereunto subscribed our names.

WILLIAM ALEXANDER DICKIE.  
WILLIAM IVAN TAYLOR.